

Nov. 25, 1924.

1,516,824

L. D. MANNES ET AL

COLOR PHOTOGRAPHY

Filed Feb. 20, 1923

2 Sheets-Sheet 1

*Fig. 1.*

Object to be Photographed



BLACK      WHITE      ORANGE-RED      BLUE-GREEN

*Fig. 2.*

Before Exposure



*Fig. 3.*

After Exposure and Development



*Fig. 4.*

After Bleaching



INVENTORS  
*Leopold D. Mannes*  
*Leopold Kosowich, Jr.*  
BY  
*James Davis Mannes Edwards*  
ATTORNEYS

Nov. 25, 1924.

1,516,824

L. D. MANNES ET AL.

COLOR PHOTOGRAPHY

Filed Feb. 20, 1923

2 Sheets-Sheet 2

*Fig. 5.* After Redevolvement of upper Layer.



*Fig. 6*  
After Toning of lower Image



*Fig. 7.*  
Finished Negative  
After Mordant- dyeing the upper Image  
COLORS & COLOR VALUES REVERSED



*Fig. 8.*  
Finished Positive  
BLACK      WHITE      ORANGERED      BLUE - GREEN  
PRINTED FROM FINISHED NEGATIVE (FIG. 7) AND TREATED SIMILARLY

INVENTORS  
Ludolf D. Mannes  
Ludolf Koslowsky, Jr.  
BY  
Pennis Davis Mann & Edmonds  
ATTORNEYS

Patented Nov. 25, 1924.

1,516,824

# UNITED STATES PATENT OFFICE.

LEOPOLD D. MANNES AND LEOPOLD GODOWSKY, JR., OF NEW YORK, N. Y.

## COLOR PHOTOGRAPHY.

Application filed February 20, 1923. Serial No. 620,269.

*To all whom it may concern:*

Be it known that we, LEOPOLD D. MANNES and LEOPOLD Godowsky, Jr., citizens of the United States, and residing in the city, 5 county, and State of New York, have invented certain new and useful Improvements in Color Photography; and we do hereby declare the following to be a full, clear, and exact description of the invention, 10 such as will enable others skilled in the art to which it appertains to make and use the same.

The present invention relates to the art 15 of color photography and has to do particularly with an improved process which may be satisfactorily employed for producing pictures commercially in substantially the colors of the original subject photographed. This application is in a sense a modification 20 or further development over the process of color photography disclosed in our co-pending application Serial No. 531,356, filed January 24th, 1922.

Color photographs are commonly produced by either a two color or a three color 25 process. The color rendition in the final picture is, of course, somewhat more complete where a three color process is employed, but for many purposes pictures 30 made according to the two color process give completely satisfactory results and present the subject photographed in substantially its natural colors.

In color photography, particularly in the 35 presentation of motion pictures, it is common to simultaneously or alternately project on the screen in superimposed relation a plurality of single color pictures equal in number to the color sensations employed, 40 the combination of the various individual pictures resulting in a composite picture containing all of the colors distributed according to their occurrence in the individual single color pictures. It has also been 45 proposed to prepare separate simultaneously taken negatives each recording a single color sensation, and to successively print them in superimposed relation on a plate or film, the prints then being colored to 50 reproduce the proper color values occurring in the original subject. The above methods are open to the objection that it is practically impossible to exactly superimpose the various individual pictures in order that 55 the resulting picture may be without color fringe or similar objectionable effect.

It has also been proposed to provide a single plate or film sensitized on one side to record a certain color sensation and sensitized on the other side for a different 60 color sensation, so that by a single exposure two images recording respectively the particular color sensations for which the coatings have been sensitized may be obtained. With this method, inasmuch as the two sensitized coatings are supported on the same 65 film, one side of the film must be specially water-proofed or otherwise protected while the image on the other side is being developed and toned. This method is further 70 limited to work in which only two exposures of different color sensations may be taken and is thus impossible of application to the three color process. As far as we are aware a process of color photography 75 employing a film or other support bearing in a substantial unitary body a plurality of sensitized emulsions to record respectively a plurality of superimposed pictures of different color sensations, has not prior to 80 our above mentioned co-pending application been successfully carried out.

It is an object of this invention to provide an improved method for producing a finished picture in substantially natural 85 colors wherein the color sensations are recorded by a single exposure and the development of the exposed film or plate is accomplished by a single operation in which the plurality of superimposed latent images are 90 completely and simultaneously developed, the developed plate or film recording the proper color values but being essentially a black and white negative which may be used for the production of ordinary black 95 and white positives in the manner of an ordinary negative.

It is another object of the invention to provide a method for satisfactorily producing colored pictures which involves the production 100 of a color negative in which the colors of the respective images are reversed, and in which the color values in each image are also reversed.

It is a further object to provide a method 105 of this nature in which the light used for printing the positives may be modified or colored to thereby improve the color rendition on the resulting positive.

It is also an object to provide a method 110 for producing color photographs which provides for correcting any inherent discrep-

ancies of internal contrast which might result from the use on the film or plate of slow and fast emulsions of different color sensitivity, to thus secure a faithful rendition of 5 the final picture in natural colors.

It is a still further object to provide a process of this character in which there is no necessity of removing or otherwise protecting a portion of the plate or film during 10 the developing process, and in which the sensitized emulsions are placed immediately adjacent at one side of the film or plate so that the respective outlines of the individual color images are exactly superimposed.

15 We have illustrated the steps of our improved process in the accompanying drawing wherein Figure 1 represents the object being photographed, the object consisting of 4 rectangular blocks colored black, white, 20 orange-red and blue-green as indicated on the drawing; Figure 2 is a transverse sectional view showing the nature of film or plate before exposure; Figure 3 is a similar view of the film or plate after exposure and 25 development; Figure 4 shows the film or plate as it appears after the bleaching operation; Figure 5 illustrates the character of the plate after the upper layer of emulsion is redeveloped; Figure 6 shows the plate 30 after toning of the lower image; Figure 7 illustrates the finished negative and Figure 8 shows the distribution of the images and colors on the finished positive.

In carrying out our improved process we 35 employ an appropriate transparent film or plate of the ordinary type and provide this plate on one surface with a plurality of sensitized coatings or emulsions as indicated in Figure 2. In a two color process two 40 emulsions are employed. The transparent film or plate is first coated with a fast silver bromide emulsion sensitized to record the red or orange-red sensations in the subject being photographed. A second coating or 45 emulsion is placed directly upon the first coating, this coating consisting of a slower silver bromide emulsion and forming with the first coating an essentially unitary layer or coating on the transparent film. This 50 second coating is sensitized for the green or greenish-blue of the spectrum. Since the blue sensation ordinarily predominates in photographic images it may be desirable to diminish the intensity of the blue rays by 55 incorporating into the upper emulsion a strong yellow dye distributed uniformly throughout the body of the emulsion. This yellow dye serves as a screen to exclude all 60 blue and violet rays from the lower emulsion and at the same time to exclude a portion of the blue light from the lower part of the upper coating and thus tone down the resulting blue-violet sensations which will be recorded in the upper emulsion.

65 In making an exposure the film of Figure

2 comprising the two superimposed emulsions forming essentially a single integral coating is supported in a camera of the ordinary type and a single exposure taken in the ordinary manner. The light entering 70 the camera first comes in contact with the emulsion sensitized for the blue-green of the spectrum, that portion of the light which passes through this emulsion serving to affect the lower layer of emulsion. Inasmuch as a lesser quantity of light acts upon the lower coating this emulsion must be fast, and the two emulsions are so constituted that a complete exposure of each will occur 75 in the same length of time. It will be understood that a compensating filter may be employed to regulate the time of exposure of either of the emulsions and in this manner a proper and complete exposure of each emulsion may be obtained without difficulty. 80 Thus, there is secured a single film with an essentially integral coating on one surface containing two exactly superimposed 85 latent images of the subject photographed, each portion of the film coating having recorded that color sensation for which it has 90 been sensitized.

While it is possible to develop the film or plate by treating the two sensitized coatings successively our invention contemplates the 95 development of the two sensitized coatings at the same time and by the same operation. For this purpose a developer, such as metol (monomethylparaminophenolsulphate) with a small alkaline content, which freely penetrates the material of the emulsions, is employed. The film is left in the developing solution until both images are completely developed whereupon the film is washed and the images fixed in the ordinary manner. 100 In our above mentioned co-pending application we have described a process contemplating the development of the upper and lower images successively, coloring each one as it is developed by chemically toning the upper 105 image and dye-mordanting the lower image. In that application we also described a process contemplating the simultaneous developing of both the upper and lower image and then suitably coloring the respective images 110 by toning the upper image and dye-mordanting the lower image in the manner above mentioned. It is to be noted that the negative resulting from the simultaneous development of the two layers of emulsions is a 115 black and white plate in which the color values of the subject photographed are correctly represented, but in which, of course, the colors themselves do not actually appear. This black and white negative may be regarded as an ordinary photographic negative 120 and may be used as desired for the production of black and white prints of the subject. The characteristics of the film or plate at this stage of the process are illus- 125 130

trated in Figure 3. It will be noted that the portion of the emulsion recording the black of the object photographed is entirely unaffected by light, while that portion recording the white of the original object is affected in both the upper and lower layers. Orange-red of the object records only in the lower layer of emulsion while the blue-green of the object records only in the upper layer. 10 This arrangement of the images formed is indicated in the figure.

After the film or plate containing the two superimposed images has been completely developed and fixed so that the black and 15 white negative results, this negative is ready for the coloring process to form a color negative from which the finished picture may be printed. Our improved process contemplates the production of a color negative by 20 first bleaching the developed images. The bleaching is accomplished by immersing the film or plate after development in a suitable bleaching solution, such as for instance a solution of potassium ferri-cyanide, and allowing 25 it to remain in the solution until both images are completely bleached. We have found that the addition of a small quantity of ammonia to the solution of potassium ferri-cyanide is advantageous and assists in 30 the producing of a proper bleaching. The effect of the potassium ferri-cyanide solution is to react on the images formed in the emulsion, converting them to silver ferro-cyanide. It will be noted that the distribution of the 35 images in the body of emulsion is identical with that of Figure 3, the only difference being that after bleaching (illustrated in Figure 4) the metallic silver of the developed images is converted to silver ferro cyanide. In 40 this step of the process there is no danger of overbleaching the images or bleaching one more than the other so that the only precaution which need be taken is to allow the plate to remain in the bleaching solution for 45 a time sufficiently long to insure complete bleaching of the images. The plate is then withdrawn from the bleaching solution and washed and dried in the usual manner.

After bleaching out the images in this 50 manner the upper image is redeveloped to its original silver state. This step is illustrated in Figure 5 wherein the images recorded in the upper layer of emulsion are converted back to metallic silver while the 55 images recorded in the lower layer are still silver ferro cyanide. This is accomplished by the use of any well-known photographic developer, a strong solution of the developer being ordinarily required, diamidophenol 60 being preferable. The plate is permitted to remain in the developing solution until the upper image, that is the image occurring in the upper strata of the emulsion on the film or plate, has been developed to its original 65 state. The developing action must, how-

ever, be checked before the lower image is affected. Inasmuch as the upper image does not extend throughout the entire thickness of the strata of emulsion sensitized to receive that image, there is an appreciable time latitude between the completion of the developing of the upper image and the beginning of the action of the developer on the lower image. The developing solution works from the surface of the emulsion down, and for 70 this reason there is ample opportunity to withdraw the plate from the developing solution after the upper image has been completely developed without experiencing a partial development of the lower image also. 75 Upon withdrawal from the developing solution the plate is, of course, washed to remove the developer. The addition of a little acetic acid to the wash water is beneficial in effecting a more thorough and complete washing 80 of the plate.

According to our invention we color the lower image, that is the image which is recorded in that portion of the emulsion originally sensitized to record the orange-red 90 sensations, blue or bluish-green, preferably bluish-green. To accomplish this the plate bearing the bleached lower image and having the upper image redeveloped, may be treated by immersing in any suitable solution containing a soluble ferrous salt, preferably ferrous chloride. The ordinary ferric chloride solution may be used, or in fact any of the solutions containing ferric salt, but we have found that there are certain disadvantages inherent in the use of solutions of this character for instance, the use of ferric chloride solution results in a certain chemical combination with the material on the plate and has a tendency to impair the 95 character of the final texture by preventing a clear transparent image being formed in the subsequent steps of the treatment to which the plate is subjected. The ferric chloride solution also exerts a slight bleaching action on the developed silver image in the upper layer of emulsion. A further effect of such a toning solution is to harden 100 the gelatine of the plate and thus increase the difficulty of washing out the plate.

To obviate these difficulties we preferably treat the bleached image with a solution of ferrous chloride. This solution gives excellent results when employed in our process and is not subject to the disadvantages and limitations incident upon the use of a ferric chloride solution. Upon immersion in such a solution the lower bleached image on the plate, which now consists of silver ferro-cyanide, reacts with the constituents of the 110 solution to form ferric or ferrous ferro-cyanide. Thus the entire lower image will be colored blue whereas the redeveloped upper image will not be affected by the acid iron solution and will, therefore, remain un- 115 120 125 130

changed. To incorporate a certain amount of green into the coloring of the lower image a soluble salt of vanadium may be added to the iron containing solution, the amount of 5 the vanadium salt added depending on the amount of green coloring which it is desired to incorporate into the image. This step is illustrated in Figure 6. After this coloring 10 operation the plate is washed and is immersed in a sodium thiosulfate solution, for the purpose of dissolving whatever soluble silver salts remain in the lower image and thus rendering the colored image clear. A 15 pure and transparent blue-green image will be obtained.

The upper image is now colored red or 20 orange-red. In carrying out this step the plate is first immersed in a suitable mordanting bath for converting the upper 25 image to a suitable mordant such as copper ferro-cyanide, silver ferro-cyanide, uranium ferro-cyanide, vanadium ferro-cyanide or the like. Our preferred mordanting solution is constituted as follows: one solution 30 (A) is prepared which consists of copper sulphate 3 grams, potassium citrate 12 grams, water 500 c. c., and a second solution (B) consisting of potassium ferri-cyanide 2½ grams, potassium citrate 12 35 grams, water 500 c. c., equal parts of solutions A and B are mixed together and the resulting mixture constitutes the mordanting bath. This bath converts the silver images in the emulsion to copper ferro-cyanide. After the mordanting of the 40 image is completed the plate is immersed in a solution of a basic aniline dye of the proper red or orange color. As is well known, the action of the mordanting bath 45 is to affect the image in such manner that it will absorb the dye according to the density of the image. This selective absorption of the dye will produce a picture colored in orange-red and having the coloring matter deposited according to the density of the image and consequently in proportion to the occurrence of the color sensations in the subject originally photographed as recorded by the emulsion. The 50 coloring of the upper image may also be accomplished by means of a selectively hardening bleach. Any of the well known bleaches of this character will be applicable for the purpose. We have obtained reasonably 55 satisfactory results with a bleach consisting of a mixture of two solutions, one of which (A) is composed of potassium ferri-cyanide 37½ grams, potassium bromide 56½ grams, potassium bichromate 37½ grams, glacial acetic acid 10 c. c., water 1000 c. c. and (B) potassium alum 60 5% solution, equal parts of solutions A and B are used. The action of such a solution is to selectively harden the gelatine and therefore 65 by cause the dye to be absorbed by the gelatine

in inverse ratio to the quantity of silver present in the image. It will be noted that when this method is employed the colors on the negative occur inversely with respect to their occurrence in the subject photographed. The finished negative is illustrated in Figure 7. The portion of the film recording the black of the object photographed is transparent while that portion recording the white of the original object bears an image in both layers of the emulsions, that is, black and white on the negative are reversed. Similarly the orange-red of the object photographed appears blue-green on the negative and is recorded in the lower layer, while the blue-green of the original object appears as an orange-red image in the negative and is recorded in the upper layer. If this method of coloring the image on the negative is employed it will also be necessary to employ a similar method when printing the positive in order that the colors in the resulting positive may be correctly represented.

It is to be noted that the colors on the negative are reversed, that is the image formed in the lower layer, which was originally sensitized to the orange-red of the spectrum, has been colored blue-green while the upper layer, originally sensitized to record blue-green values, has been colored orange-red. The negative plate is complete and presents two images in a pure and transparent condition, with the colors incorporated properly throughout. The plate is essentially a negative. Thus black in the subject photographed appears white on the plate, and likewise white appears black. This reversal of the white and black values in each of the superimposed images is in addition to the interchanging of the orange-red and blue-green in the respective layers of emulsion.

A similar process is employed in printing the positive. The plate of film which is to receive the positive is similar in all respects to the negative plate before exposure and bears the same kind of emulsions arranged in the same manner upon the transparent support. The positive is exposed once, and after exposure is treated in a manner in all respects similar to the process employed in producing the color negative. It will be noted that the colors must again be reversed in the printing of the positive in order that correct representations will be obtained in the finished picture. The finished positive is illustrated in Figure 8 and by comparison of this figure with Figure 7 which shows the completed negative, it will be seen that a reversal of color values is effected in the printing of the positive. The negative thus bears color values reversed with respect to the occurrence of colors in the object photographed

and the finished positive bears color values reversed with respect to the occurrence of the colors in the negative. The result is that the finished positive is a true representation of the object photographed.

The reversal of the colors in forming the negative and the second reversal of the colors in forming the positive has several advantages probably the most notable of which is that the color reversal serves to compensate for any inherent discrepancy of internal contrast in slow and fast emulsions. The layer of emulsion nearest the film must, of course, be a fast emulsion, while the upper layer, which is directly exposed to the light must be slower in order that a complete exposure of both emulsions can be obtained in the same length of time. By interchanging the colors on the color negative and again reversing them during the printing of the positive the possibility of undesirable results which might occur were one color carried throughout in a single emulsion are avoided.

In our co-pending application mentioned above we describe a method of producing a photograph in three colors by employing a film bearing three emulsions sensitized respectively to different colors. For instance, the lower or first coating might be red sensitive, the middle coating green sensitive, and the upper coating blue sensitive, and having incorporated it in a quantity of yellow dye in the same manner that such dye is incorporated into the upper emulsion as described in this application. We prefer, however, to carry out the three color process by exposing a second ordinary plate to record the blue sensations and make from it a yellow print in the positive to supply the third color. This yellow positive may be printed as a separate print or may be incorporated directly upon the plate already bearing the positive in two colors.

Our invention also contemplates an improvement in printing the positive from the color negative by means of which improvement we secure a better distinction and a more vigorous coloring of the positive. To accomplish this we employ a dichroic filter having transmission bands at the extreme ends of the spectrum to accentuate the color separation of the negative. By thus coloring the light used for printing the positive we have found that a very good rendition of colors is obtained on the positive even when the colors of the negative are not of exceptional purity.

It is to be understood that with our improved process there is no possibility of a color fringe occurring in the picture inasmuch as the various images are exactly superimposed. Likewise the requisite manipulation is simplified in that the development of the plurality of superimposed images is

accomplished simultaneously and by a single operation, there being no need for separating or otherwise protecting the various images during the process. We have described certain preferred embodiments of our invention, but it is to be understood that certain modifications, such as varying the exact nature of the different developing and toning solutions employed, and the like, may be made within the full scope of the appended claims, and it is also to be understood that the plate or film used in the specification and claims is not intended to refer to any particular type of photographic film, plate or the like, but is to be understood to mean any suitable support bearing a sensitized medium which may be used as a sensitive element in the production of the pictures.

Claims.

1. A method of producing a color photograph comprising forming in layers of emulsion sensitized respectively to record different color values, a plurality of superimposed latent images of different color sensations, developing said latent images and coloring the images thus developed respectively in colors other than those whose values are recorded in the said respective images.

2. A method of producing a color photograph comprising forming in layers of emulsion sensitized respectively to record different color values, a plurality of superimposed latent images of different color sensations, developing said latent images and coloring each of the respective images thus developed with a color whose values are recorded by another of said images.

3. The method of producing a color photograph in two colors comprising forming in layers of emulsion sensitized respectively to record different color values and combined to constitute a substantially unitary body, two superimposed latent images of different color sensations, simultaneously developing and then fixing said two images and then coloring each of said images with that color whose values are recorded by the other image.

4. The method of producing a color photograph in two colors comprising forming in layers of emulsion sensitized respectively to record different color values, two superimposed latent images of different color sensations, simultaneously developing and then fixing said two images, bleaching both images, then re-developing the upper image and then coloring each of said images with that color whose values are recorded by the other image.

5. The method of producing a color photograph in two colors comprising forming in layers of emulsion provided on one side of a single support to constitute a sub-

- stantially unitary body and sensitized respectively to record different color values, two superimposed latent images of different color sensations, simultaneously developing and then fixing said two images, bleaching both images, redeveloping the upper image and then coloring the negative by first coloring the lower image and then mordanting and coloring the upper image.
10. The method of producing a color photograph in two colors comprising forming in layers of emulsion sensitized to record different color values and combined to form a substantially unitary body of sensitized media, two superimposed latent images of different color sensations, simultaneously developing and then fixing said two images, bleaching both images, redeveloping the upper image and then coloring the negative by first coloring the lower image with a color for which the upper portion of the said medium was originally sensitized, then mordanting the upper image and then coloring the upper image with that color for which the lower portion of the said medium was originally sensitized.
15. 7. The method of producing a color photograph in two colors comprising forming in layers of emulsion sensitized to record different color values and combined to form a substantially unitary body, two superimposed latent images of different color sensations, simultaneously developing and then fixing said two images, bleaching both images, then redeveloping the upper image and then coloring the negative by first chemically toning the lower image and then by dye-toning the upper image.
20. 8. The method of producing a color photograph comprising forming at a single exposure in layers of emulsion sensitized to record respectively different color values and combined to form a substantial unitary body of sensitized medium, a plurality of superimposed images, the upper image recording the blue-green sensations of the subject photographed and the lower image recording the orange-red sensations, simultaneously developing and then fixing the two images, bleaching both images to thereby convert both images into silver ferrocyanide, redeveloping the upper image and then coloring the lower image blue-green and mordanting and coloring the upper image orange-red to form a color negative.
25. 9. The method of producing a color photograph comprising forming in layers of emulsion sensitized respectively to record different color values, a plurality of superimposed latent images of different color sensations, developing said latent images, bleaching both images, redeveloping the upper image and coloring each image with that color whose values are recorded in the other image, thereby forming a color negative.
30. 10. The method of producing a color photograph in two colors comprising forming in layers of emulsion sensitized to record different color values and combined to form a substantially unitary body of sensitized medium two superimposed latent images, simultaneously developing and then fixing said two images, bleaching both images and then redeveloping the upper image, coloring the lower image, coloring the upper image in that color for which the lower image bearing strata of said medium was sensitized by relatively hardening with an appropriate bath the gelatine containing the said upper image in proportion to the density of the image, then treating the plate with a suitable dye solution whereby the dye will be absorbed in inverse ratio to the quantity of silver present in the upper image to thus form a color negative.
35. 11. The method of producing a color photograph comprising forming in suitably sensitized media a plurality of superimposed latent images of different color sensations, developing said images and coloring each image with that color whose values are recorded in the other image thereby forming a color negative, printing a positive from said color negative with light passing through a dichroic filter to thereby separate bands of color transmission corresponding to the colors of the two images, the image constituting said positive being recorded in layers of emulsion sensitized respectively to record different color values.
40. 12. The method of producing a color photograph in two colors comprising forming in layers of emulsion sensitized respectively to record different color values two superimposed latent images of different color sensations, simultaneously developing and then fixing said two images, bleaching both images, redeveloping the upper image, then coloring each of said images with that color whose values are recorded by the other image, producing a second ordinary plate to record the blue sensations in the subject photographed and forming therefrom in the positive a yellow image.
45. 13. The method of producing a color photograph comprising forming in layers of emulsion sensitized respectively to record different color values and combined to form a substantial unitary body of sensitized medium at a single exposure a plurality of

superimposed images, the upper image recording the blue-green sensations of the subject photographed and the lower image recording the orange-red sensations, simultaneously developing and then fixing the two images, bleaching both images, redeveloping the upper image and then coloring the lower image blue-green and mordanting and coloring the upper image orange-red to form a color negative.

14. A method of color photography comprising forming a plurality of superimposed

images of different color sensations in layers of emulsion sensitized respectively to record different color values, developing and then bleaching said images, redeveloping one of said images and then toning the other of said images in its bleached condition with a solution of ferrous chloride.

In testimony whereof we affix our signatures.

LEOPOLD D. MANNES.  
LEOPOLD GODOWSKY, JR.